

May 19, 1953

H. A. GOLWYNNE

2,638,627

# METHOD AND APPARATUS FOR THE PRODUCTION OF METAL POWDER

Filed Sept. 29, 1949



*INVENTOR.*

HENRY A. GOLWYNNE

BY

<sup>b7</sup>  
Pennie, Edmonds, Morton & Barrows

**ATTORNEYS**

## UNITED STATES PATENT OFFICE

2,638,627

## METHOD AND APPARATUS FOR THE PRODUCTION OF METAL POWDER

Henry A. Golwynne, New York, N. Y.

Application September 29, 1949, Serial No. 118,625

19 Claims. (Cl. 18—2.5)

1

This invention relates to the production of metal powder and has for its object certain improvements in the method of and apparatus for producing metal powder.

In my copending applications, Ser. Nos. 118,621 and 118,622, filed September 29, 1949, simultaneously herewith I have disclosed and claimed a method of and apparatus for producing metal powder involving the atomizing of molten metal with a blast of inert gas, freezing the atomized metal into finely divided particles and recovering the resulting metal powder. In accordance with the method, the molten metal atomizing, metal powder forming and powder separating steps are conducted in a confined main circulatory system filled with inert gas continuously circulating therethrough under a pressure higher than atmospheric to prevent ingress of outside air. And, in accordance with the apparatus, the improvement comprises a confined circulatory system adapted to be filled with gas under pressure higher than atmospheric, the system includes a gasometer to hold surplus gas and to take care of expansion and contraction of the gas, a chamber for atomizing molten metal and chilling atomized molten metal into powder, a blower for circulating the gas around the system, and a separator for separating the powder from the gas.

Although a continuous current of gas is passed through the atomizing and powder forming zones in the chamber, there is a tendency for an appreciable amount of the newly formed powder to settle to the bottom of the chamber. While clean-out openings may be provided at the bottom of the chamber through which to remove such precipitated powder, the opening of the clean-outs reduces the gas pressure in the system to atmospheric pressure, so that outside air may readily enter. As pointed out in the copending applications, every precaution is taken to prevent ingress of outside air because of its oxygen and nitrogen, which form oxides and nitrides that adhere to the atomizing nozzle and tend to clog its gas ports and molten metal outlet. The use of such clean-out openings also introduces a serious fire or explosion hazard because the passage of air into the atomizing and powder forming zones of the chamber provides an environment conducive to combustion of the metal powder, particularly magnesium powder, etc.

My investigations have led to the discovery that a chamber may be provided and operated in such a manner as to overcome for the most part disadvantages of the kind enumerated. The atomizing and powder forming steps may be conducted

2 without interruption as the newly formed metal powder is promptly and effectively removed from the chamber.

In accordance with the method of the invention, the molten metal atomizing and metal powder forming steps are conducted in a confined zone filled with cool inert gas continuously passing therethrough under a pressure higher than atmospheric to prevent ingress of outside air. A continuous current of additional inert gas is advantageously injected into the lowermost portion of the zone to help keep the powder particles in suspension in the gas passing through the zone.

According to the invention, the apparatus comprises a chamber with an inlet for the entrance of a continuous current of gas and an outlet for the continuous withdrawal of the gas with the newly formed metal powder particles suspended therein. In an advantageous practice, the bottom of the chamber is provided with one or more openings for the injection of a continuous current of additional inert gas to help keep the powder particles in suspension in the current of gas passing through the chamber.

According to a presently preferred practice, the atomizing and powder forming steps are conducted in an elongated zone with the gas entering at one end and the gas laden with metal powder leaving at the other end. Spaced streams of additional inert gas are passed into the bottom of the elongated zone, the entrance of the streams being spaced from one another in the general elongated direction of travel of the current of gas in the zone so that the streams of additional gas tend to sweep along the bottom portions of the zone between adjacent stream entrances to help keep the bottom of the zone free of precipitated metal powder and to keep the powder in suspension in the gas passing through the zone.

Similarly an apparatus is provided for such conduct of the method. To this end, the chamber may be divided into an upper compartment for the atomizing and powder forming steps and a lower compartment for supplying additional gas to the upper compartment, the upper compartment being provided with an inlet for the entrance of a continuous current of inert gas and an outlet for the continuous withdrawal of the gas with newly formed metal powder particles suspended therein. The lower compartment is in turn provided with a separate inlet for the entrance of a continuous supply of gas. A plurality of spaced openings is disposed between the top of the lower compartment and the bottom of the upper compartment for the passage of a plurality

of streams of the additional gas from the lower to the upper compartment, the openings being spaced from one another in the general direction of travel of the current of gas in the upper compartment between the inlet and the outlet so that the streams of gas passing through the openings help keep the powder particles in suspension in the gas passing through the upper compartment. The openings preferably extend in the general direction of travel of the gas in the upper compartment so that the streams passing through the openings tend to sweep along the bottom portions of the upper compartment between adjacent openings to help keep the bottom free of precipitated metal powder.

These and other features of the invention will be better understood by referring to the accompanying drawing, taken in conjunction with the following description, in which:

Fig. 1 is a diagrammatic side elevation in section of an apparatus illustrative of a practice of the invention; and

Fig. 2 is a cross-sectional view on the line 2—2 of Fig. 1.

The apparatus shown comprises a main tank or chamber 10 provided at opposite ends with similar bonnets 12 and 14. Furnace bonnets 16 and 18 are secured or securable to chamber bonnets 12 and 14. An atomizer 20 for molten metal extends from furnace bonnet 16 into chamber bonnet 12 and a similar atomizer 22 extends from furnace bonnet 18 into chamber bonnet 14. These may be regarded as conventional atomizers in which a stream of molten metal is blasted with inert gas. An inlet conduit 30 for relatively cool inert gas connects with the top of chamber bonnet 12 and a similar inlet conduit 32 connects with the top of chamber bonnet 14. As pointed out in my co-pending applications, these conduits, as well as the main tank or chamber, form part of the main circulatory system. A continuous supply of relatively cool inert gas is passed through either or both conduits into the chamber for the purpose of chilling the atomized metal and carrying away the newly formed metal powder. While molten metal could be atomized simultaneously at both ends of the chamber, in practice it is usually confined to one end, preferably the one to the right, so that the direction of the stream of molten metal to be atomized and the direction of the gas passing through the chamber are concurrent. While needed repairs are made to the furnace at that end, it is advantageous to continue operations with a furnace at the other end.

An outlet conduit 36 for the passage of gas laden with newly formed powder connects the lower end of the chamber, to the left with the suction side of a blower 38 provided with an outlet conduit 40 on its pressure side leading to one or more powder-gas separators, etc., as disclosed, for example, in my co-pending applications. An inlet conduit 44 for the supply of additional amounts of cool inert gas connects with the lower end of the chamber, to the right. This conduit supplies extra gas to help keep the newly formed metal powder in suspension in the current of gas passing through the chamber toward the blower. These conduits form part of the main circulatory system, as pointed out in my co-pending applications.

As more particularly shown in Fig. 2, the cylindrical tank is divided essentially into an upper compartment 50, which is in the form of a trough, a lower compartment 52, which is essen-

tially in the form of a duct; and two side compartments 54 and 56, which are seated from each other as well as from the other two compartments. All of the compartments extend longitudinally of the chamber. The upper and lower compartments are tapered in reverse order. Thus, upper compartment 50 has its smallest cross-section at the right end of the tank, and its largest cross-section at the left end. The lower compartment or gas distributing duct 52, on the other hand, has its largest cross-section at the right end, where the gas is shown to enter, and its smallest cross-section at the left end.

The compartments are obtained by the use of opposed pairs of butt-welded plates 61 to 68, top plates 71 to 78 and a pair of spaced side plates 81 and 82. They are suitably welded to the cylindrical wall and to each other to provide an integral structure. Plates 61 to 68 are pitched or slanted at an angle, toward the bottom of the trough, so that powder settling thereon will tend to slide down into the bottom of the trough. Referring for a moment to Fig. 1, it will be seen that an overlying lip 84 is welded to the head of the cylindrical tank at the right end to provide a slot 86 between inlet conduit 44 and upper compartment 50. Similar underlying lips 88, 90, 91, 92, 93, 94 and 95 provide slots 100 to 106. Upper plate 71 of the duct is spaced above the bottom of the tank to provide a similar slot 107 at the left end of the tank, in direct communication with outlet conduit 36. The overlying and underlying lips are sufficiently long to cause gas passing therethrough to sweep along the bottom of the upper compartment. In other words, gas going through slot 86 sweeps along the top of plate 78, gas passing through slot 100 sweeps across the top of plate 78, gas passing through slot 100 sweeps across the top of plate 71, etc.

A gas blow-off 110 is provided along the top of the tank as a safety measure. In case of an explosion the blow-off releases the pressure thus preventing damage to the chamber. Inlets 120 connect conduit 44 with the side compartments and outlets 121 connect the side compartments with outlet 36. While the side compartments are normally sealed from each other and the other compartments, it is possible for leaks to develop at the welded joints. It is therefore desirable to have an arrangement which will permit the side compartments to be cleared of air and filled with inert gas, as well as to equalize the pressures between compartments.

The apparatus may be operated as follows: After chamber or tank 10, as well as the entire confined main circulatory system, is filled with purified inert gas, for example as described in the copending applications, a continuous current of inert gas under pressure higher than atmospheric is passed through the system, including inlet conduit 30, upper compartment 50, and outlet conduit 36. The circulation is obtained by the use of blower 38, the suction side of which connects the outlet side of the chamber. Inlet conduit 32 is closed and atomizer 22 is not in operation. With atomizer 20 in operation a fine stream of molten magnesium issuing therefrom is blasted with inert gas to atomize the metal. The atomized metal is promptly enveloped and frozen into powder particles in the relatively cool inert gas sweeping through the upper compartment.

While the newly formed particles of magnesium powder tend to remain in suspension in the

gas as the gas passes through the chamber to the blower, some of it also tends to settle by gravity onto plates 61 to 68 and toward the bottom or base of the trough of the upper compartment. Additional amounts of relatively cool inert gas are, therefore, introduced into the upper compartment by way of inlet conduit 44. According to a present practice, the amount of gas entering the upper compartment by way of inlet 44 and lower compartment or duct 52 substantially exceeds that entering by way of inlet 30. Some of the gas from inlet 44 issues as a relatively small stream through slot 86, the stream being directed along the top of plate 78 at the bottom of the trough. Any magnesium powder settling or tending to settle on that plate is, therefore, swept up and placed in suspension in the main and large current of gas passing through the upper compartment. In a similar manner gas in the lower compartment or duct passes as a stream through slot 100 along the top of plate 77 at the bottom of the trough of the upper compartment. Similar streams of gas pass through slots 101 to 106, so that plates 76, 75, 74, 73, 72 and 71 at the bottom of the trough of the upper compartment are continuously swept with streams of gas under sufficient velocity to keep the powder from settling and to keep it in suspension. An additional stream of inert gas passes through duct 107 into the discharge end of the upper compartment. Some of the gas thus introduced through the slots also spreads to the side and sweeps across plates 61 to 68 to keep them clean of powder. The mixture of gas and powder is under a great deal of turbulence which inhibits settling of the powder. The powder laden gas is in effect sucked from the upper compartment by the blower and blown to gas-powder separators (not shown), where the powder is recovered. If the molten magnesium is to be atomized at the other end of the chamber, or tank, inlet conduit 30 and atomizer 20 are not in operation. A fine stream of molten magnesium issuing from the nozzle of atomizer 22 is blasted with inert gas and the atomized metal is promptly enveloped in the relatively cool inert gas entering the upper compartment by way of inlet conduit 32. The force behind the fine stream of molten metal issuing from the nozzle of the atomizer and the force of the inert gas used to atomize the stream of molten metal is sufficient to throw the atomized metal substantially across the length of the chamber. Additional amounts of inert gas are fed into the upper compartment, as just described, through ducts 86 and 100 to 107.

While various inert or non-reactive gases may be employed, helium is at present the most readily available. The method and apparatus may be used to produce various metal powders, either in elemental or alloy form. They are at present being used to produce magnesium powder and also magnesium-aluminum alloy powders.

It will be clear to those skilled in this art that the method and apparatus of the invention readily lend themselves to various useful modifications. The chamber or tank can, for example, be placed in numerous positions, horizontal, inclined, or vertical. The chamber can be arranged in any suitable form. Various arrangements are possible for introducing the additional amount of inert gas to the atomizing and powder-forming zone. Whatever the particular arrangement selected, the newly formed particles of metal powder are kept in suspension so that pow-

der laden gas may be promptly and efficiently and continuously removed from the chamber.

I claim:

1. In the method of producing metal powder by atomizing molten metal with a blast of gas inert to the metal and freezing the atomized metal into finely divided particles in a zone forming a part of a main circulatory system, the improvement which comprises conducting the molten metal atomizing and metal powder forming steps in a main stream of the inert gas moving continuously from the main circulatory system through the zone, the gas being under sufficient pressure higher than atmospheric to prevent ingress of outside air and sufficiently cool to chill the atomizing metal into powder particles, introducing into the zone continuously an auxiliary stream of inert gas from the main circulatory system to help keep the newly formed metal powder in suspension in the zone, and withdrawing the metal powder continuously while still suspended in the main stream of inert gas leaving the zone.
2. Method according to claim 1, in which the auxiliary stream of inert gas from the main circulatory system is fed into the lowermost portion of the zone to help keep the powder particles in suspension in the gas passing through the zone.
3. Method according to claim 1, in which spaced auxiliary streams of the inert gas from the main circulatory system are passed into the lowermost portion of the zone to help keep the powder particles in suspension in the gas passing through the zone.
4. Method according to claim 1, in which spaced auxiliary streams of the inert gas from the main circulatory system are passed into the zone in the general direction of travel of the gas in the zone to help keep the powder particles in suspension in the gas passing through the zone.
5. Method according to claim 1, in which spaced auxiliary streams of the inert gas from the main circulatory system are passed into the zone in the general direction of travel of the gas so that the streams of gas tend to sweep along the bottom portions of the zone between adjacent streams to help keep the bottom of the zone free of precipitated metal powder and to keep the powder in suspension in the gas passing through the zone.
6. Method according to claim 1, in which the zone is elongated with inert gas entering at one end and gas from the main circulatory system laden with metal powder leaving at the other end, and spaced auxiliary streams of the inert gas are passed into the bottom of the elongated zone, the entrance of the streams being spaced from one another in the general elongated direction of travel of the gas in the zone so that the streams of gas tend to sweep along the bottom portions of the zone between adjacent stream entrances to help keep the bottom of the zone free of precipitated metal powder and to keep the powder in suspension in the gas passing through the zone.
7. In apparatus for producing metal powder by atomizing molten metal with a blast of gas inert to the metal and freezing the atomized metal into finely divided particles in a chamber forming part of a main circulatory system, the improvement comprising an inlet in the chamber connecting the main circulatory system for the entrance of a continuous main stream of the inert gas and an outlet in the chamber connecting the main circulatory system for the continu-

ous withdrawal of the main stream of the gas with the newly formed metal powder particles suspended therein and a separate inlet connecting the main circulatory system with the chamber for introducing an auxiliary stream of inert gas from the main circulatory system to help keep the newly formed powder particles suspended in the main stream of inert gas passing through the chamber.

8. Apparatus according to claim 7, in which the separate inlet is provided at the bottom of the chamber for the injection of the auxiliary stream of inert gas into the lowermost portion of the chamber to help keep the powder particles in suspension in the main stream of gas passing through the chamber.

9. Apparatus according to claim 7, in which spaced openings are provided at the bottom of the chamber for the injection of spaced streams of additional inert gas from the main circulatory system into the lowermost portion of the chamber to help keep the powder particles in suspension in the gas passing through the chamber.

10. Apparatus according to claim 7, in which spaced openings are provided at the bottom of an elongated chamber, the openings being spaced from one another and directed in the general direction of travel of the current of gas through the chamber so that the streams of additional gas injected through the openings into the chamber tend to sweep along the bottom portions to help keep the bottom free of precipitated metal powder and to keep the powder in suspension in the gas passing through the chamber.

11. Apparatus according to claim 7, in which the chamber is divided into an upper compartment for the atomizing and powder forming steps and a lower compartment for supplying the additional gas to the upper compartment; the upper compartment is provided with said first mentioned inlet and outlet; the lower compartment is provided with a separate inlet for the entrance of the auxiliary stream of gas; and a plurality of spaced openings are disposed between the top of the lower compartment and the bottom of the upper compartment for the passage of a plurality of streams of the gas from the lower to the upper compartment to help keep the powder particles in suspension in the main stream of gas passing through the upper compartment.

12. Apparatus according to claim 7, in which the chamber is divided into an upper compartment for the atomizing and powder forming steps and a lower compartment for supplying additional gas to the upper compartment; the upper compartment is provided with said first mentioned inlet and outlet; the lower compartment is provided with the separate inlet for the entrance of the auxiliary stream of gas; and a plurality of spaced openings are disposed between the top of the lower compartment and the bottom of the upper compartment for the passage of a plurality of streams of the gas from the lower to the upper compartment; said openings being spaced from one another in the general direction of travel of the gas in its upper compartment between the inlet and outlet so that the streams of gas passing through the openings help keep the powder particles in suspension in the gas passing through the upper compartment.

13. Apparatus according to claim 7, in which

75 the chamber is elongated; the chamber is divided into an elongated upper compartment for the atomizing and powder forming steps and an elongated lower compartment for supplying additional gas to the upper compartment; the upper compartment is provided with said first mentioned inlet and outlet at opposite ends; the lower compartment is provided with the separate inlet for the entrance of the auxiliary stream of gas; and a plurality of spaced openings are disposed between the top of the lower compartment and the bottom of the upper compartment for the passage of a plurality of streams of the gas from the lower to the upper compartment; said openings being spaced from one another in the general direction of travel of the gas in the upper compartment between its inlet and outlet so that the streams of gas passing through the openings help keep the powder particles in suspension in the gas passing through the upper compartment.

14. Apparatus according to claim 7, in which the chamber is divided into an upper compartment for the atomizing and powder forming steps and a lower compartment for supplying additional gas to the upper compartment; the upper compartment is provided with said first mentioned inlet and outlet; the lower compartment is provided with the separate inlet for the entrance of the auxiliary stream of gas; and a plurality of spaced openings are disposed between the top of the lower compartment and the bottom of the upper compartment for the passage of a plurality of streams of the gas from the lower to the upper compartment; said openings extending in the general direction of travel of the gas in the upper compartment between its inlet and the outlet so that the streams of gas passing through the openings tend to sweep along the bottom portions of the upper compartment between adjacent openings to help keep the bottom free of precipitated metal powder and to keep the powder in suspension in the gas passing through the upper compartment.

15. Apparatus according to claim 7, in which the chamber is elongated; the chamber is divided into an upper elongated compartment for the atomizing and powder forming steps and a lower elongated compartment for supplying additional gas to the upper compartment; the upper compartment is provided with said first mentioned inlet and outlet at opposite ends; the lower compartment is provided with the separate inlet for the entrance of a continuous current of gas; and a plurality of spaced openings are disposed between the top of the lower compartment and the bottom of the upper compartment for the passage of a plurality of streams of the gas from the lower to the upper compartment; said openings being spaced from one another in the general elongated direction of travel of the gas in the upper compartment between its inlet and outlet so that the streams of gas passing through the openings will tend to sweep along the bottom portions of the upper compartment between adjacent openings to help keep the bottom portions free of precipitated metal powder and to keep the powder in suspension in the gas passing through the upper compartment.

16. In apparatus for producing metal powder by atomizing molten metal with a blast of gas and freezing the atomized metal into finely divided particles in a chamber, the improvement comprising an elongated chamber substantially the

same in cross section throughout its length, the chamber being divided into an upper elongated compartment for the atomizing and powder forming steps and a lower elongated compartment for supplying additional gas to the upper compartment, an inlet at one end of the upper compartment for the entrance of a continuous current of gas and an outlet at the other end of the upper compartment for the continuous withdrawal of the gas with the newly formed metal powder particles suspended therein, the upper compartment tapering from the inlet end to the outlet end with the largest cross section at the inlet end and the smallest cross section at the outlet end, an inlet in the lower compartment for the entrance of a continuous current of gas, the lower compartment tapering in a reverse direction from that of the upper compartment with its largest cross section opposite the inlet end of the upper compartment and its smallest cross section opposite the outlet end of the upper compartment, and a plurality of spaced openings disposed between the top of the lower compartment and the bottom of the upper compartment for the passage of a plurality of streams of the gas from the lower to the upper compartment, said openings being spaced from one another in the general direction of travel of the gas in the upper compartment between its inlet and outlet so that the streams of gas passing through the openings

30

help keep the powder particles in suspension in the gas passing through the upper compartment.

17. Apparatus according to claim 16, in which the upper compartment is in the form of a trough and the spaced openings are in the bottom of the trough.

18. Apparatus according to claim 16, in which the openings are spaced from one another in the general elongated direction of travel of the gas in the upper compartment between its inlet and outlet so that the streams of gas passing through the openings will tend to sweep along the bottom portions of the upper compartment between the adjacent openings to help keep the bottom portions free of precipitated metal powder and to keep the powder in suspension in the gas passing through the upper compartment.

19. Apparatus according to the preceding claim, in which the upper compartment is in the form of a trough and the spaced openings are in the bottom of the trough.

HENRY A. GOLWYNNE.

References Cited in the file of this patent

UNITED STATES PATENTS

| Number    | Name    | Date          |
|-----------|---------|---------------|
| 1,156,079 | Holley  | Oct. 12, 1915 |
| 2,255,227 | Parsons | Sept. 9, 1941 |
| 2,402,441 | Paddle  | June 18, 1946 |